# EUROPEAN PATENT SPECIFICATION

(11) **EP 4 594 452 B1**
(45) Date of publication and mention of the grant of the patent: **10.12.2025**
(21) Application number: 24828782.3
(22) Date of filing: 13.12.2024
(51) Int. Cl.: C10M 169/04, C10M 145/16, C10M 149/06

(54) **A PYROLYSIS OIL WITH REDUCED POUR POINT AND/OR VISCOSITY**
PYROLYSEÖL MIT REDUZIERTEM STOCKPUNKT UND/ODER VISKOSITÄT
HUILE DE PYROLYSE À POINT D'ÉCOULEMENT ET/OU VISCOSITÉ RÉDUITS

(30) Priority: 21.12.2023 EP 23219217
(43) Date of publication of application: 06.08.2025
(73) Proprietor: Evonik Operations GmbH, 45128 Essen (DE)
(72) Inventor: SIRAK, Sofia, Plymouth Meeting, Pennsylvania 19462 (US); MEISTER, Claudia, 64285 Darmstadt (DE); WAGH, Sachin Subhash, 64289 Darmstadt (DE)
(74) Representative: Evonik Patent Association
(86) International application number: PCT/EP2024/086138
(87) International publication number: WO 2025/132054

(56) References cited:
- US-A1- 2022 081 634
- US-B2- 10 738 138

## Description

### TECHNICAL FIELD OF THE INVENTION

The invention relates to a composition comprising a pyrolysis oil and a polymeric additive for reducing the pour point, viscosity, or both the pour point and viscosity of the pyrolysis oil. The invention further relates to a method of manufacturing said composition, the use of a polymeric additive for reducing the pour point, viscosity, or both the pour point and viscosity of a pyrolysis oil. The invention further relates to a method for transporting or storing a pyrolysis oil.

### BACKGROUND OF THE INVENTION

Plastic production continues to grow rapidly, and plastic products remain to be a crucial part of our lives due to the versatility of the material and the low cost associated with plastic production. It is estimated that 250 million tons of plastic per year are either landfilled or dispersed into the environment. It is also predicted that the use of plastic will continue to increase in the future. The increase in plastic production will also be associated with the increase in associated plastic waste, especially with single-use plastic items. The increase in plastic waste has also brought interest in how to effectively recycle or convert plastic waste back into usable materials.

One effective way to treat plastic waste is by thermochemically converting plastic waste via a pyrolysis process. Pyrolysis is a thermal cracking process that occurs in the absence of oxygen at temperatures above 400°C. The process breaks down polymer chains into smaller chains and molecules. The pyrolysis process can therefore convert plastic waste material into usable products thereby addressing the plastic waste management issues. There are many types of plastics, but the majority of plastic waste is made up of low-density polyethylene (LDPE), high density polyethylene (HDPE), polypropylene (PP), polyvinylchloride (PVC), polystyrene (PS), and polyethylene terephthalate (PET). Of those plastics, polyethylene and polypropylene constitute the greatest portion of plastic waste. The pyrolysis provides a final product termed in the art 'pyrolysis oil'. The main products produced from plastic pyrolysis include liquid oil, wax, solid residues, and gas. All such residues are then processed further as part of existing plastic processing plants or steam crackers used in refineries.

In the pyrolysis process, the conversion of plastic to usable materials, e.g. oil, gas, and wax, is dependent on several factors. The most influential factors are the reactor design, the process temperature, the type of plastic used, and the type of catalyst.

The wax residue comprises those pyrolysis products having alkyl chains of 16 or more carbon atoms. The wax residue is a valuable product in the pyrolysis process. The amount of wax residue produced can greatly influence the final pyrolysis oil properties. The main driver in the amount of wax residue produced is the plastic feedstock being introduced into the pyrolysis process. For example, olefinic plastics such as polyethylene and polypropylene are more linear polymers, which therefore break down into waxy linear alkyl chains when converted in the pyrolysis process. Pyrolysis oils produced from polyethylene and polypropylene can yield over 50wt% wax residue depending on the specific pyrolysis oil process conditions.

Specific process conditions including catalyst types can also influence oil-to-wax ratio. To obtain a lower wax residue content in the final product, certain catalysts can be used. Also, conditions such as residence time in the reactor can be influential. For example, 'fast' pyrolysis leads to the production of waxy hydrocarbon mixtures, whereas 'slow' pyrolysis typically produces more oil than wax. (Materials 2021, 14, 2586).

However, waxy chains can also cause a variety of transportation and storage issues. The waxy chains of 12 or more carbon atoms can begin to crystallize as the pyrolysis oil cools to ambient temperature after the pyrolysis process. Pyrolysis oils also typically have a large quantity of paraffins with waxy chains of 16 to more than 40 carbon atoms. These wax chains are most problematic since the melting point is much higher. The wax crystals can then build up and cause an increase in viscosity, making the thicker oil more difficult to pump or move. If there is enough wax residue in the pyrolysis oil, especially in polyolefin pyrolysis oils, then the wax crystals may cause the entire product to solidify at lower temperatures heading towards ambient temperature. Once solidified, expensive heating must be used to melt the product in order to move or process it further. The wax crystals may also clog equipment such as filters and pipelines, thus increasing servicing costs. Lastly, high wax amounts can lead to paraffin deposition on pipelines in the production lines. As wax builds up, the efficacy and lifetime of the equipment is decreased.

Despite this, wax is a valuable pyrolysis product, and existing plastic processing plants have been designed and built to use the wax residue. However, the wax residue made in the pyrolysis process, especially from increasingly used olefin feedstocks, is making transportation and storage of the pyrolysis oil more difficult and more expensive.

As previously explained, the amount of wax residue varies depending on the plastic feedstock used, and the specific process conditions. And, polyolefin-based pyrolysis oils produced via current or standard pyrolysis processes, tend to produce the most amount of wax, which therefore have the most problems, especially at ambient conditions. The 'pour point' is the lowest temperature at which the pyrolysis oil will still flow, and pyrolysis oils with high wax residue have relatively high pour points (for example, above 50°C), which are usually above standard operating conditions and storage temperatures. This leads to difficulty in processing such pyrolysis oils, as the oil may solidify and become unable to transport. Heat is typically applied to the oil to liquefy it for storage and transportation. This expends heat energy and takes time. Therefore, even slight reductions in the pour point could drastically reduce the amount of heat energy expended and time taken to liquefy or to keep in liquid form the pyrolysis oil for transportation and storage.

One solution for reducing the pour point of the pyrolysis oil is to change the process conditions or the catalysts type to produce pyrolysis oils with lower pour points. But to do this, expensive catalysts need to be employed, the processes must run longer, or special reactors are required. Increasing process times or changing the reactor also increases the cost or decreases the overall efficiency. Furthermore, the valuable wax product is no longer produced at the same amount, and so cannot be available for subsequent processing set up to expect the wax product. Other solutions have been implemented to isolate the wax by introducing a dewaxing step and reprocessing the oil to crack the wax into smaller molecules. However, these solutions also add costs and decrease efficiency to the process.

US2012/0310023A1 discloses that oils obtained in pyrolysis of polyolefin containing plastics mixtures are frequently wax-like semisolid products, and that the use of specific catalysts can result in the production of more light and less waxy products.

Lee et al. in the Journal of Analytical and Applied Pyrolysis 94 (2012) 209-214 explain that most of the plastic waste consisting of polyethylene is mainly converted in waxy oils. The waxy oils can be problematic because they could result in a breakdown of plant operations, ranging from pipeline blockages to shorter instrument life cycles. Thus, upgrading technology for pyrolysis to produce high-quality oils is needed. The authors demonstrated the efficacy of zeolite catalysts in the catalytic upgrading of the pyrolysis process.

Hakeem et al. in Applied Petrochemical Research (2018) 8:203-210 describe the problem with higher wax contents in pyrolysis oils and propose that catalysis could also be used to reduce the amount of wax in the final products and upgrade the oil to a lower wax quality in order to improve final properties.

KR100994244B1 discloses the need to remove the wax from the process and proposes the use of a separation device for wax removal. Therefore, the pyrolysis process will require an additional step to the process.

US2022/081634 discloses the use of a polymeric additive for improving the cold flow properties of a plastic-derived synthetic feedstock composition (see [0008]). Among the disclosed polymeric additives, the polymer can be a copolymer of an alpha-olefin monomer with an ethylenically unsaturated carboxylic acid monomer or derivatives thereof, such as maleic anhydride monomer with a range of weight-average molecular weight from 20,000 to 70,000 g/mol (see [0070], [0076] and example 3 of Table 1). This document is focused on the treatment of plastic pyrolysis oil with a high wax residue content of alkanes with long carbon chains (high content of waxes having C₁₆ or longer carbon chains - see e.g. [0048], [0086], [0097], [0115], [00127], as well as the two treated pyrolysis oils of the experimental part [0153]).

WO2023/183460 discloses a composition comprising a pyrolysis oil and an additive composition comprising (a) one or more nitrogen containing antioxidants; and optionally, (b) a copolymer comprising maleic anhydride derived units and α-olefin derived units; and/or (c) the reaction product of a carboxylic acid and a polyamine. It also relates to a method of improving the oxidation stability of a composition comprising a pyrolysis oil by adding to the composition the above-indicated additive composition (see abstract). The optional copolymer comprising maleic anhydride derived units and alpha-olefin derived units, has preferably a number average molecular weight of from 1,000 to 50,000 g/mol, more preferably from 8,000 to 17,000 g/mol (pages 12-14 and copolymer C of Table 1 with a Mₙ of 15,000 g/mol).

Jin et al. in the Chinese Journal of Chemical Engineering 26 (2018) 400-406 explain that reactor design can help influence the wax quantity in the final pyrolysis oil product. The authors studied falling film reactor in comparison to other reactor types to improve the liquid/wax ratio. The authors showed that the liquid wax ratio in the vertical falling film pyrolysis reactor is slightly higher than that achieved in the tubular reactor, equal to that in the rotary kiln reactor, and slightly lower than that in the medium fluidized bed.

Thus, as exemplified above, the conventional solutions to reduce viscosity and pour point of pyrolysis oils have been to reduce or eliminate production of the wax by changing the reactor design, adding special catalyst, increasing processing times or having an additional dewaxing process step. Although those methods help in producing liquid pyrolysis oils with a lower wax content, it creates additional costs, maintenance work, increased processing times, which decrease production efficiency and are thus not good industrially viable solutions. Furthermore, the industry looks for high wax residue content pyrolysis oils for cracking processes, without having the transportation and storage disadvantages.

However, the properties of the plastic pyrolysis oils strongly depend on the production process, which leads to plastic pyrolysis oils having different wax residue content of alkanes. Therefore, there is still a need to investigate further to find effective and cost-efficient solutions for the treatment of plastic pyrolysis oils from a plastic pyrolysis process in order to keep them liquid, improving the transport and storage of these oils before the cracking process.

The present invention is therefore directed to provide a pyrolysis oil with a lower pour point, lower viscosity or both lower pour point and viscosity, as well as other objectives.

### BRIEF SUMMARY OF THE INVENTION

The invention is defined in the appended claims.

According to a first aspect of the invention there is provided a composition comprising a plastic pyrolysis oil a) and a polymeric additive b), for reducing the pour point, viscosity, or both the pour point and viscosity of the pyrolysis oil.

According to a second aspect of the invention there is provided a method of manufacturing the composition of the first aspect of the invention comprising the steps of:
providing a plastic feedstock;
pyrolyzing the plastic feedstock to generate a plastic pyrolysis oil a);
preparing a polymeric additive b) as described herein; and
adding polymeric additive b) to the pyrolysis oil a).

According to a third aspect of the invention there is provided the use of a polymeric additive b), as described herein to reduce the pour point of a plastic pyrolysis oil a), or to reduce the viscosity of the pyrolysis oil, or both.

According to a fourth aspect of the invention there is provided a method of transporting or storing a plastic pyrolysis oil a) comprising the step of adding a polymeric additive b) to the pyrolysis oil to form the composition of the first aspect of the invention

### DETAILED DESCRIPTION OF THE INVENTION

According to the invention, there is provided a composition comprising a plastic pyrolysis oil a) and a polymeric additive b), wherein the polymeric additive b) is a copolymer P) prepared by polymerizing a monomer composition comprising
i) 10 to 70 % by weight of monomers selected from alkyl maleate compound of Formula (I), maleimide compound of Formula (II) or a mixture thereof, based on the total weight of the copolymer P), wherein R" in Formula (I) and Formula (II) is a linear or branched alkyl group having from 10 to 40 carbon atoms, preferably from 10 to 30 carbon atoms, more preferably from 12 to 30 carbon atoms, even more preferably from 18 to 22 carbon atoms; and
ii) 30 to 90 % by weight of a non-functionalized alpha-olefin of Formula (III) or a mixture thereof, based on the total weight of the copolymer P), wherein R₂ is a linear alkyl group having from 8 to 40 carbon atoms, preferably from 10 to 40 carbon atoms, more preferably from 15 to 35 carbon atoms, even more preferably from 20 to 32 carbon atoms, and
wherein the plastic pyrolysis oil a) comprises 12 % by weight or less of n-paraffin waxes with C₁₆ or longer carbon chains, based on the total weight of the plastic pyrolysis oil a).

The polymeric additive b) reduces the pour point of the pyrolysis oil. The polymeric additive may also reduce the viscosity of the pyrolysis oil. The polymeric additive may also reduce both the pour point and the viscosity of the pyrolysis oil.

Preferably, the pour point of a pyrolysis oil a) is reduced by at least 1 °C, more preferably by at least 2 °C, even more preferably by at least 3 °C, most preferably by at least 5 °C, by the addition of the polymeric additive as described herein, when compared to the same pyrolysis oil with no polymeric additive.

The reduction in viscosity is preferably of at least 10 %, preferably at least 20 %, even more preferably 30 %, 40 %, 50 %, or 60 % or more, at a temperature from -20 °C to +80 °C, preferably from -10 °C to +50 °C, when the polymeric additive is added to the pyrolysis oil with a wax residue as described herein, when compared to the same pyrolysis oil with no polymeric additive.

The polymeric additive b) has a wax inhibition of greater than 1 % relative to the pyrolysis oil a) as determined by the cold finger test measured using CF-15 cold finger device manufactured by PSL with rack temperature set at 5 °C above the Wax Appearance Temperature (WAT) and finger temperature set 20 °C below the WAT for a test period of 24 hours as described in detail in the experimental part of the present invention. The wax inhibition is preferably greater than 5 %, 10 %, 15 %, 25 % or 30 % (measured according to the cold finger test described above and more detail in the experimental part).

### Plastic pyrolysis oil a)

The term "plastic pyrolysis oil" or "pyrolysis oil" as used herein includes any pyrolysis oil produced from the pyrolysis of plastics or plastic waste. Pyrolysis is a thermal cracking process that occurs in the complete or substantial absence of oxygen, at temperatures above 250 °C to convert plastic into energy, in the form of solid, liquid and gaseous fuels. The process breaks down polymer chains into smaller chains and molecules.

The plastic pyrolysis oil is preferably a plastic waste pyrolysis oil, namely a pyrolysis oil produced from plastic waste. The pyrolysis of plastic waste with a thermal degradation of plastic waste at different temperatures (300-900 °C), to produce liquid oil is for example described in Rehan et al., 2017, Int. Biodeterior. Biodegrad. 119, 162-175.

Preferably, the plastic pyrolysis oil is a plastic pyrolysis oil and/or a plastic waste pyrolysis oil, wherein the plastic and plastic waste are both selected from polyolefins, more preferably polylolefins selected from high-density polyethylene (HDPE), low-density polyethylene (LDPE), polypropylene (PP) and a mixture thereof; polyethylene terephthalate (PET); polyvinyl chloride (PVC); polystyrene (PS); or a mixture thereof.

The term "polyolefin pyrolysis oil" and "polyolefin waste pyrolysis oil" as used herein defines an oil produced from the pyrolysis of polyolefins or waste polyolefin respectively, wherein the plastic and plastic waste are selected from high-density polyethylene (HDPE), low-density polyethylene (LDPE) and polypropylene (PP).

Pyrolysis oils having a wax content of at least 1 % by weight typically have problems regarding storage and transportation, due to the high pour point and high viscosity of the pyrolysis oil. The terms "wax residue" or "wax content" include that portion of the pyrolysis oil that comprises linear hydrocarbons containing 16 or more carbon atoms.

In the context of the present invention, the term "linear hydrocarbons containing 16 or more carbon atoms" used herein means "n-paraffin waxes with C₁₆ or longer carbon chains", namely, "n-paraffin waxes being a mixture of C₁₆ to C₁₉ n-paraffin waxes, C₂₀ to C₂₉ n-paraffin waxes, C₃₀ to C₃₉ n-paraffin waxes, and n-paraffin waxes with C₄₀ or longer carbon chains".

The pyrolysis oil a) of the composition of the present invention has a wax residue of 12 % by weight or less of n-paraffin waxes with C₁₆ or longer carbon chains, preferably from 0.01 % by weight to 12 % by weight of n-paraffin waxes with C₁₆ or longer carbon chains, more preferably from 0.05 % by weight to 12 % by weight of n-paraffin waxes with C₁₆ or longer carbon chains. The pyrolysis oil a) of the composition of the present invention may also preferably have a wax residue of 10 % by weight or less of n-paraffin waxes with C₁₆ or longer carbon chains, more preferably from 0.01 % to 10 % by weight of n-paraffin waxes with C₁₆ or longer carbon chains, even more preferably from 0.05 % by weight to 10 % by weight of n-paraffin waxes with C₁₆ or longer carbon chains based on the total weight of the plastic pyrolysis oil a).

According to a preferred embodiment of the invention, the plastic pyrolysis oil a) preferably comprises from 0 % to 12 % by weight of C₁₆ to C₁₉ n-paraffin waxes, from 0 % to 12 % by weight of C₂₀ to C₂₉ n-paraffin waxes, from 0 % to 12 % by weight of C₃₀ to C₃₉ n-paraffin waxes, and from 0 % to 12 % by weight of n-paraffin waxes with C₄₀ or longer carbon chains, wherein the total wax content of n-paraffin waxes with C₁₆ or longer carbon chains sums up to 12 % by weight or less, based on the total weight of the plastic pyrolysis oil.

According to a preferred embodiment of the invention, the plastic pyrolysis oil a) preferably comprises from 0 % to 12 % by weight of C₁₆ to C₁₉ n-paraffin waxes, from 0 % to 12 % by weight of C₂₀ to C₂₉ n-paraffin waxes, from 0 % to 12 % by weight of C₃₀ to C₃₉ n-paraffin waxes, and from 0 % to 12 % by weight of n-paraffin waxes with C₄₀ or longer carbon chains, wherein the total wax content of n-paraffin waxes with C₁₆ or longer carbon chains sums up from 0.01 to 12 % by weight, based on the total weight of the plastic pyrolysis oil.

According to another preferred embodiment of the invention, the plastic pyrolysis oil a) preferably comprises from 0 % to 10% by weight of C₁₆ to C₁₉ n-paraffin waxes, from 0 % to 10 % by weight of C₂₀ to C₂₉ n-paraffin waxes, from 0 % to 10 % by weight of C₃₀ to C₃₉ n-paraffin waxes, and from 0 % to 10 % by weight of n-paraffin waxes with C₄₀ or longer carbon chains, wherein the total wax content of n-paraffin waxes with C₁₆ or longer carbon chains sums up to 10 % by weight or less, based on the total weight of the plastic pyrolysis oil.

According to another preferred embodiment of the invention, the plastic pyrolysis oil a) preferably comprises from 0 % to 10% by weight of C₁₆ to C₁₉ n-paraffin waxes, from 0 % to 10 % by weight of C₂₀ to C₂₉ n-paraffin waxes, from 0 % to 10 % by weight of C₃₀ to C₃₉ n-paraffin waxes, and from 0 % to 10 % by weight of n-paraffin waxes with C₄₀ or longer carbon chains, wherein the total wax content of n-paraffin waxes with C₁₆ or longer carbon chains sums up from 0.01 to 10 % by weight, based on the total weight of the plastic pyrolysis oil.

Advantageously, reducing or lowering the pour point or the viscosity or both of a pyrolysis oil makes it easier to transport and store a pyrolysis oil having a wax residue. In this way, the present invention obviates the current requirements to modify the reactor, or to modify the reaction process (for example, by the addition of a catalyst) when processing a pyrolysis oil having a wax residue that it is desired to maintain. In this way, current plastic processing plants designed to expect the use of a wax residue pyrolysis oil can continue to operate without redesign.

### Polymeric additive b)

The polymeric additive b) is a copolymer P) prepared by polymerizing a monomer composition comprising
i) from 10 to 70 % by weight of monomers selected from alkyl maleate compound of Formula (I), maleimide compound of Formula (II) or a mixture thereof, based on the total weight of the copolymer P), wherein R" in Formula (I) and Formula (II) is a linear or branched alkyl group having from 10 to 40 carbon atoms; and
ii) from 30 to 90 % by weight of one or more non-functionalized alpha-olefin of formula (III), based on the total weight of the copolymer P), wherein R₂ is a linear alkyl group having from 8 to 40 carbon atoms, preferably from 10 to 40 carbon atoms, more preferably from 15 to 35 carbon atoms, even more preferably from 20 to 32 carbon atoms.

According to the present invention, the polymeric additive b) is one polymer P), or a mixture of one or more polymer P).

Within the context of the present invention, the monomer composition corresponds to the total amount of monomers to prepare the copolymer P).

In a preferred embodiment, the polymeric additive b) is a copolymer P) prepared by polymerizing a monomer composition comprising
i) 10 to 70 % of alkyl maleate compound of Formula (I), based on the total weight of the copolymer, and
ii) 30 to 90 % by weight of one or more non-functionalized alpha-olefin of formula (III), based on the total weight of the copolymer P).

Preferably R" in Formula (I) and Formula (II) is a linear or branched alkyl group having from 10 to 40 carbon atoms, more preferably from 12 to 30 carbon atoms, even more preferably from 18 to 22 carbon atoms.

Preferably R₂ in Formula (III) is a linear alkyl group having from 10 to 40 carbon atoms, more preferably from 10 to 35 carbon atoms, even more preferably from 10 to 32 carbon atoms.

The content of alkyl maleate i) in the copolymer P) is preferably from 20 to 50 % by weight, more preferably from 25 to 40% by weight, based on the total weight of the copolymer P).

The content of alpha-olefin ii) in the copolymer P) is preferably from 50 to 80 % by weight, more preferably 60 to 75 % by weight, based on the total weight of the copolymer P).

In one embodiment the polymeric additive b) is a polymer prepared by polymerizing a monomer composition comprising C₁₈-C₂₂ alkyl maleate and C₂₀-C₃₂ non-functionalized alpha-olefin.

In another embodiment, the polymeric additive b) is a polymer prepared by polymerizing a monomer composition comprising C₁₈-C₂₂ alkyl maleate and C₂₀-C₂₄ non-functionalized alpha-olefin.

In a further embodiment, the polymeric additive b) is a polymer prepared by polymerizing a monomer composition comprising C₁₈-C₂₂ alkyl maleate and C₁₀-C₁₈ non-functionalized alpha-olefin.

A copolymer is a polymer formed from two or more different types of monomers linked in a polymeric chain.

According to the present invention, the polymeric additive b) is one polymer P), or a mixture of one or more polymer P). Preferably, the polymeric additive b) comprises one or more copolymers P), even more preferably copolymers P) selected from the group consisting of a polymer prepared by polymerizing a monomer composition comprising C₁₈-C₂₂ alkyl maleate and C₂₀-C₃₂ non-functionalized alpha-olefin, a polymer prepared by polymerizing a monomer composition comprising C₁₈-C₂₂ alkyl maleate and C₂₀-C₂₄ non-functionalized alpha-olefin, a polymer prepared by polymerizing a monomer composition comprising C₁₈-C₂₂ alkyl maleate and C₁₀-C₁₈ non-functionalized alpha-olefin, or a mixture thereof.

As used herein, the term "maleate" refers to esters of maleic acid. The term "alkyl maleate" refers to esters of maleic acid and aliphatic alcohols. The alkyl maleate described herein are characterized by the number of carbon atoms in the alkyl chain derived from the alcohol.

For example, the term "C₁₈-C₂₂ alkyl maleate" refers to esters of maleic acid and linear or branched alcohols having 18 to 22 carbon atoms. The term encompasses individual maleic esters with an alcohol of a particular length, and likewise a mixture of maleic esters with alcohols of different lengths. Likewise, the term "C₂₀-C₂₄ alkyl maleate" refers to esters of maleic acid with linear or branched alkyl chain having 20 to 24 carbon atoms. The term encompasses individual maleic esters with an alcohol of a particular length, and likewise mixtures of maleic esters with alcohols of different lengths.

Alpha-olefin is compound made up of hydrogen and carbon that contains one or more pairs of carbon atoms linked by a double bond. As used herein, the term C₁-C₄₀ olefin, C₁₀-C₁₈ olefin or C₂₀-C₃₂ olefin refers to an olefin comprising a linear, branched or cyclic residue with 1 to 40 carbon atoms, 10 to 18 carbon atoms or 20 to 32 carbon atoms, respectively.

As an optional component, the monomer composition to prepare the copolymer P) may contain further monomer iii) derived from one or more comonomers, or a mixture thereof.

Preferably, these comonomers iii) are selected from the list consisting of:
hydroxyalkyl (meth)acrylates, preferably hydroxyalkyl (meth)acrylates selected from 3-hydroxypropyl (meth)acrylate, 3,4-dihydroxybutyl (meth)acrylate, 2-hydroxyethyl (meth)acrylate, 2 hydroxypropyl (meth)acrylate, 2,5-dimethyl-1,6-hexanediol (meth)acrylate, 1,10 decanediol (meth)acrylate;
aminoalkyl (meth)acrylates and aminoalkyl (meth)acrylamides, preferably aminoalkyl (meth)acrylates and aminoalkyl (meth)acrylamides selected from N-(3-dimethyl-aminopropyl)methacrylamide, 3-diethylaminopentyl (meth)acrylate, 3-dibutyl-aminohexadecyl (meth)acrylate;
nitriles of (meth)acrylic acid and other nitrogen-containing (meth)acrylates, preferably nitriles of (meth)acrylic acid and other nitrogen-containing (meth)acrylates selected from N-(methacryloyloxyethyl)diisobutylketimine, N-(methacryloyloxyethyl)dihexadecyl-ketimine, (meth)acryloylamidoacetonitrile, 2-methacryloyloxyethylmethylcyanamide, cyanomethyl (meth)acrylate;
aryl (meth)acrylates like benzyl (meth)acrylate or phenyl (meth)acrylate, where the acryl residue in each case can be unsubstituted or substituted up to four times;
carbonyl-containing (meth)acrylates, preferably carbonyl-containing (meth)acrylates selected from 2-carboxyethyl (meth)acrylate, carboxymethyl (meth)acrylate, N-methyacryloyloxy)-formamide, acetonyl (meth)acrylate, N-methacryloyl-2 pyrrolidinone, N-(2-methyacryloxyoxyethyl)-2-pyrrolidinone, N-(3-methacryloyloxy-propyl)-2-pyrrolidinone, N-(2-methyacryloyloxypentadecyl(-2-pyrrolidinone, N-(3 methacryloyloxyheptadecyl-2-pyrrolidinone;
(meth)acrylates of ether alcohols, preferably (meth)acrylates of ether alcohols selected from tetrahydrofurfuryl (meth)acrylate, methoxyethoxyethyl (meth)acrylate, 1-butoxypropyl (meth)acrylate, cyclohexyloxyethyl (meth)acrylate, propoxyethoxyethyl (meth)acrylate, benzyloxyethyl (meth)acrylate, furfuryl (meth)acrylate, 2-butoxyethyl (meth)acrylate, 2-ethoxy-2-ethoxyethyl (meth)acrylate, 2-methoxy-2-ethoxypropyl (meth)acrylate, ethoxylated (meth)acrylates, 1-ethoxybutyl (meth)acrylate, methoxyethyl (meth)acrylate, 2-ethoxy-2-ethoxy-2-ethoxyethyl (meth)acrylate, esters of (meth)acrylic acid and methoxy polyethylene glycols;
(meth)acrylates of halogenated alcohols, preferably (meth)acrylates of halogenated alcohols selected from 2,3-dibromopropyl (meth)acrylate, 4 bromophenyl (meth)acrylate, 1,3-dichloro-2-propyl (meth)acrylate, 2-bromoethyl (meth)acrylate, 2-iodoethyl (meth)acrylate, chloromethyl (meth)acrylate;
oxiranyl (meth)acrylate, preferably oxiranyl (meth)acrylate selected from 2, 3-epoxybutyl (meth)acrylate, 3,4-epoxybutyl (meth)acrylate, 10,11 epoxyundecyl (meth)acrylate, 2,3-epoxycyclohexyl (meth)acrylate, oxiranyl (meth)acrylates such as 10,11-epoxyhexadecyl (meth)acrylate, glycidyl (meth)acrylate;
phosphorus-, boron- and/or silicon-containing (meth)acrylates, preferably phosphorus-, boron- and/or silicon-containing (meth)acrylates selected from 2-(dimethyl-phosphato)propyl (meth)acrylate, 2-(ethylphosphito)propyl (meth)acrylate, 2 dimethylphosphinomethyl (meth)acrylate, dimethylphosphonoethyl (meth)acrylate, diethylmethacryloyl phosphonate, dipropylmethacryloyl phosphate, 2 (dibutylphosphono)ethyl (meth)acrylate, 2,3-butylenemethacryloylethyl borate, methyldiethoxymethacryloylethoxysiliane, diethylphosphatoethyl (meth)acrylate;
sulfur-containing (meth)acrylates, preferably sulfur-containing (meth)acrylates selected from ethylsulfinylethyl (meth)acrylate, 4-thio-cyanatobutyl (meth)acrylate, ethylsulfonylethyl (meth)acrylate, thiocyanatomethyl (meth)acrylate, methylsulfinylmethyl (meth)acrylate, bis(methacryloyloxyethyl) sulfide;
heterocyclic (meth)acrylates, preferably heterocyclic (meth)acrylates selected from 2-(1-imidazolyl)ethyl (meth)acrylate, oxazolidinylethyl (meth)acrylate, N-methacryloylmorpholine and 2-(4-morpholinyl)ethyl (meth)acrylate;
maleic acid and maleic acid derivatives, preferably mono- and diesters of maleic acid, maleic anhydride, methylmaleic anhydride, maleinimide, methylmaleinimide;
fumaric acid and fumaric acid derivatives, preferably mono- and diesters of fumaric acid;
vinyl halides, preferably vinyl halides selected from vinyl chloride, vinyl fluoride, vinylidene chloride and vinylidene fluoride;
vinyl esters, preferably vinyl acetate;
vinyl monomers containing aromatic groups, preferably vinyl monomers containing aromatic groups selected from styrene, substituted styrenes with an alkyl substituent in the side chain, such as alpha-methylstyrene and alpha-ethylstyrene, substituted styrenes with an alkyl substituent on the ring such as vinyltoluene and p-methylstyrene, halogenated styrenes such as monochlorostyrenes, dichlorostyrenes, tribromostyrenes and tetrabromostyrenes;
heterocyclic vinyl compounds, preferably heterocyclic vinyl compounds selected from 2-vinylpyridine, 3-vinylpyridine, 2-methyl-5-vinylpyridine, 3-ethyl-4-vinylpyridine, 2,3-dimethyl-5-vinylpyridine, vinylpyrimidine, vinylpiperidine, 9-vinylcarbazole, 3-vinylcarbazole, 4-vinylcarbazole, 1-vinylimidazole, 2-methyl-1-vinylimidazole, N-vinylpyrrolidone, 2-vinylpyrrolidone, N-vinylpyrrolidine, 3-vinylpyrrolidine, N-vinylcaprolactam, N-vinylbutyrolactam, vinyloxolane, vinylfuran, vinylthiophene, vinylthiolane, vinylthiazoles and hydrogenated vinylthiazoles, vinyloxazoles and hydrogenated vinyloxazoles;
vinyl and isoprenyl ethers;
methacrylic acid and acrylic acid, or a mixture thereof.

In an embodiment, the comonomer iii) is styrene.

As used herein, the term "(meth)acrylate" refers to esters of acrylic and methacrylic acid, and to mixtures thereof. The term "alkyl (meth)acrylate" refers to esters of (meth)acrylic acid and aliphatic alcohols. The alkyl (meth)acrylates described herein are characterized by the number of carbon atoms in the alkyl chain derived from the alcohol.

The proportion of comonomers in the monomer composition can vary depending on the use and property profile of the polymeric additive b). Preferably, the content of comonomer iii) in the monomer composition to prepare the copolymer P) is in the range from 0 to 20 % by weight, preferably from 0 to 15 % by weight, more preferably from 0.1 to 15 % by weight, based on the total weight of the monomer composition.

Preferably, the amounts of monomers and comonomers sum up from 95 to 100 % by weight, more preferably sum up to 100 % by weight, based on the total weight of the monomer composition.

Preferably, the weight-average molecular weight of the polymeric additive b) is from 8,000 to 600,000 g/mol, preferably from 8,000 to 300,000 g/mol even more preferably from 8,000 to 100,000 g/mol and most preferably from 10,000 to 50,000 g/mol, determined by gel permeation chromatography using poly(methylmethacrylate) calibration standards according to DIN 55672-1 (as described in more details below).

### Preparation process for polymeric additive b)

Preparation of olefin-co-ester of maleic acid and olefin-co-imide-derivative of maleic acid are well known in the art and described in literature such as in US10738138B2 and US4192930.

Olefin-co-ester of maleic acid polymer: These polymers include are a combination of one or more olefins and an ester of maleic acid or a maleic acid derivative such as citraconic acid, nadic acid. Such polymers can be made by copolymerizing an unsaturated ester of maleic anhydride (or a derivative thereof) with one or more alpha-olefins or by reacting an alcohol (a hydroxyl-bearing moiety) with a copolymer of maleic anhydride (or a derivative thereof) and one or more alpha-olefins.

R" represents the alkyl group from the alcohol or hydroxy bearing moiety used to create the ester of maleic anhydride. Depending on the esterification conversion, the R" group may appear once or twice in the maleic anhydride derivative portion of the polymer.

The term alkyl maleate refers to esters of maleic acid or a maleic acid derivative. The structure is represented by Formula (I).

"C₁₈-C₂₂ alkyl maleate" refers to esters of maleic acid or a maleic acid derivative where the alkyl chain length is 18-22 carbon atoms. The esterification of the maleic anhydride can be partial or full and R" in Formula (I) is a linear or branched alkyl group having from 18 to 22 carbon atoms.

Olefin-co-imide-derivative of maleic acid polymers: These polymers are a combination of one or more olefins and an N-alkyl, N-aryl, or N-alkaryl maleimide or maleimide derivative. Such polymers may be made by copolymerizing an unsaturated imide with one or more alpha-olefins, or reacting an amine with a copolymer of maleic anhydride (or a derivative thereof) and one or more alpha-olefins.

The term alkyl maleimide refers to derivatives of the reaction of maleic anhydride and ammonia or an amine derivative. The structure is represented by Formula (II).

"C₁₈-C₂₂ alkyl maleimide" refers to refers to derivatives of the reaction of maleic anhydride and ammonia or an amine derivative. The imidization of the maleic anhydride can be partial or full and R" in Formula (II) is a linear or branched alkyl group having from 18 to 22 carbon atoms.

The polymers of the polymeric additive b) can be obtained by free-radical polymerization and related processes, for example ATRP (Atom Transfer Radical Polymerization), RAFT (Reversible Addition Fragmentation Chain Transfer) or NMP processes (nitroxide-mediated polymerization). More preferably, the polymers b) of the invention are prepared by free-radical polymerization.

Customary free-radical polymerization is described, inter alia, in Ullmann's Encyclopedia of Industrial Chemistry, Sixth Edition. In general, a polymerization initiator is used for this purpose. The usable initiators include the azo initiators widely known in the technical field, such as 2,2'-azo-bis-isobutyronitrile (AIBN), 2,2'-azo-bis-(2-methylbutyronitrile) (AMBN) and 1,1-azobiscyclohexanecarbonitrile, and also peroxy compounds such as methyl ethyl ketone peroxide, acetylacetone peroxide, dilauryl peroxide, tert-butyl peroxypivalate, tert-butyl peroxy-2-ethylhexanoate, tert-amyl peroxy-2-ethylhexanoate, ketone peroxide, tert-butyl peroctoate, methyl isobutyl ketone peroxide, cyclohexanone peroxide, dibenzoyl peroxide, tert-butyl-peroxybenzoate, tert-butyl-peroxyisopropylcarbonate, 2,5-bis(2-ethylhexanoyl-peroxy)-2,5-dimethylhexane, tert-butyl-peroxy-2-ethylhexanoate, tert-butyl-peroxy-3,5,5-trimethylhexanoate, dicumyl peroxide, 1,1-bis(tert-butyl-peroxy)cyclohexane, 1,1-bis(tert-butyl-peroxy)-3,3,5-trimethylcyclohexane, cumyl hydroperoxide, tert-butyl-hydroperoxide, bis(4-tert-butylcyclohexyl) peroxydicarbonate, or a mixture of two or more of the aforementioned compounds with one another, and mixtures of the aforementioned compounds with compounds which have not been mentioned but can likewise form free radicals. Preferred initiator for the preparation of polymeric additive b) is tert-butyl-peroxy-2-ethylhexanoate.

Furthermore, a chain transfer agent can be used. It is well-known in the art that a good way to control the molecular weight of a polymer chain is to use chain transfer agents during the polymerization synthesis. Chain transfer agents are molecules with a weak chemical bond which facilitate the chain transfer reaction. During the chain transfer reaction, the radical of the polymer chain abstracts a hydrogen from the chain transfer agent, resulting in the formation of a new radical on the sulfur atom of the chain transfer agent capable of further propagation. Common chain transfer agents are organic compounds comprising SH groups such as n-butyl mercaptan, n-octyl mercaptan, n-dodecyl mercaptan, tert-dodecyl mercaptan, butylthiol glycolate, and octylthiol glycolate. A preferred chain transfer agent is selected from n-dodecyl mercaptan, tert-dodecyl mercaptan or a mixture thereof, most preferably n-dodecyl mercaptan.

Preferably, the monomer mixture to prepare the polymeric additive b) of the present invention may comprise 0.05 to 7 % by weight, preferably 0.05 to 5 % by weight and more preferably 0.1 to 1 % by weight of initiator based on the total weight of the monomer composition to prepare the polymeric additive b). The amount of chain transfer agents to prepare the polymeric additive b) is in the range of 0 to 5 % by weight, preferably 0.01 to 5 % by weight and more preferably 0.05 to 4 % by weight, based on the total weight of the monomer composition.

The polymerization may be carried out at standard pressure, reduced pressure or elevated pressure. The polymerization temperature is not critical. Conventionally the polymerization temperature may be in the range of 0 °C to 200 °C, preferably 0 °C to 140 °C, and more preferably 60 °C to 130 °C.

The polymerization may be carried out with or without solvent. The term solvent is to be understood here in a broad sense. The polymerization is preferably carried out in a nonpolar solvent. These include hydrocarbon solvents, for example aromatic solvents such as toluene, benzene and xylene, saturated hydrocarbons, for example cyclohexane, heptane, octane, nonane, decane, dodecane, which may also be present in branched form, or a mixture thereof, such as naphtha. These solvents may be used individually and as a mixture. Particularly preferred solvents are mineral oils, diesel fuels of mineral origin, naphthenic solvents, natural vegetable and animal oils, biodiesel fuels and synthetic oils (e.g. ester oils such as dinonyl adipate), or a mixture thereof.

### Plastic pyrolysis oil composition according to the invention

Preferably, the composition comprises polymeric additive b) at a concentration of from 0.001 % by weight to 1 % by weight of polymeric additive b), based on the total weight of the pyrolysis oil composition. More preferably, the composition comprises polymeric additive b) at a concentration of from 0.005 % by weight to 0.8 % by weight of polymeric additive b), based on the total weight of the pyrolysis oil composition. Even more preferably, the composition comprises polymeric additive b) at a concentration of from 0.005 % by weight to 0.5 % by weight of polymeric additive b), based on the total weight of the pyrolysis oil composition.

In specific embodiments, the plastic pyrolysis oil is a polyolefin pyrolysis oil, wherein the pyrolysis oil is produced at least partially from the pyrolysis of one or more polyolefins. Optionally, the pyrolysis oil a polyethylene and/or polypropylene pyrolysis oil, wherein the pyrolysis oil is produced at least partially from the pyrolysis of polyethylene and/or polypropylene.

Preferably, pyrolysis oil a) and polymeric additive b) sum up from 90 to 98 % by weight, based on the total weight of the pyrolysis oil composition.

The composition according to the invention may further comprise an additive c), wherein additive c) is any of the group comprising scale inhibitors, corrosion inhibitors, oxygen scavengers, biocides, emulsion breakers, antifoam agents, drag reducing agents, hydrate inhibitors, paraffin dispersants, asphaltene control agents, a pour point depressant other than copolymer P), or a mixture thereof.

Preferably, then the amounts of compounds a), b), c) sum up to 90 to 99 % by weight, more preferably sum up to 95 to 98 % by weight, even more preferably sum up to 100 % by weight, based on the total weight of the composition.

Any specific embodiments or preferred aspects of the polymeric additive b), polymer P) and pyrolysis oil a), as listed herein, apply to the plastic pyrolysis oil composition according to the invention.

### Preparation of the plastic pyrolysis oil composition according to the invention

The invention also provides a method of manufacturing a composition, as described above, comprising the steps of:
providing a plastic feedstock;
pyrolyzing the plastic feedstock to generate a plastic pyrolysis oil a);
preparing a polymeric additive b); and
adding polymeric additive b) to the plastic pyrolysis oil a).

The method for preparing the plastic pyrolysis oil composition according to the invention preferably comprises the step of mixing the pyrolysis oil and the polymeric additive. More preferably, the method comprises the step of mixing for at least 5, 10, 15, 25 or 30 minutes.

The method may also comprise a step of heating the pyrolysis oil and the polymeric additive, preferably to at least 40 °C, even more preferably to at least 50 °C, most preferably to at least 60 °C. The method may comprise heating and mixing the pyrolysis oil simultaneously.

The method of the present invention is able to reduce the pour point of the pyrolysis oil, or to reduce the viscosity of the pyrolysis oil, or to achieve both. The resulting pyrolysis oil is thereby easier to transport and store compared to the pyrolysis oil with no polymeric additive. In addition, no modifications to plant design are required to provide a pyrolysis oil having a reduced pour point or viscosity, as this can be achieved by adding the polymeric additive of the present invention after the pyrolysis oil is made.

In specific embodiments, the method comprises the step of providing a plastic feedstock comprising one or more polyolefins and producing the pyrolysis oil at least partially from said feedstock. The polyolefins may be polyethylene and/or polypropylene.

### Use of the polymeric additive b)

The present invention also extends to the use of a polymeric additive as defined herein to reduce the pour point of a plastic pyrolysis oil or to reduce the viscosity of the pyrolysis oil, or to do both.

Preferably, the pour point of a pyrolysis oil is reduced by at least 1 °C, more preferably by at least 2 °C, even more preferably by at least 3 °C, most preferably by at least 5 °C, by the addition of the polymeric additive as described herein, when compared to the same pyrolysis oil with no polymeric additive.

The reduction in viscosity is preferably of at least 10, preferably 20 or 30, even more preferably 40, 50, or 60 % or more, at a temperature from 0 to 80 °C, preferably at either 40 °C, 45 °C or 50 °C, or at a temperature from 40 to 50 °C, when the polymeric additive is added to the pyrolysis oil with a wax residue as described herein, when compared to the same pyrolysis oil with no polymeric additive.

### Method for transporting or storing a plastic pyrolysis oil

Advantageously, as exemplified in the experimental part, the composition according to the invention has a lower pour point and viscosity in comparison to untreated pyrolysis oils. Pyrolysis oils usually solidify making them difficult to transport. In contrast, pyrolysis oils with lower pour point will remain liquid at lower temperatures, thus making them easier to transport and heat does not need to be applied to the composition before transportation and storage.

The present invention also extends to a method of transporting or storing a plastic pyrolysis oil a) comprising the step of adding a polymeric additive b) to the pyrolysis oil to form the composition described herein.

By reducing the pour point of the pyrolysis oil comprising a wax residue of 12 % by weight or less of n-paraffin waxes with C₁₆ or longer carbon chains, or by reducing the viscosity of such pyrolysis oil, or doing both, the manufacturer or user of the pyrolysis oil can maintain current transportation or storage conditions of pyrolysis oils having a total wax content of 12 % by weight or less of n-paraffin waxes with C₁₆ or longer carbon chains, based on the total weight of the plastic pyrolysis oil, by using their existing plant design, or possibly lower the transportation or storage conditions of high or higher wax residue pyrolysis oils using existing plant design, i.e. reduced OPEX.

The present invention provides a method for transporting or/and storing a plastic pyrolysis oil a) in liquid form at a temperature in the range -20 °C to +50 °C.

In the context of the present invention, all details provided herein above on the composition, pyrolysis oil and polymeric additive do also apply for the method according to the invention.

### EXPERIMENTAL PART

The invention is further illustrated in detail hereinafter with reference to examples and comparative examples, without any intention to limit the scope of the present invention.

### Methods

In the present invention, the weight-average molecular weights (M_{w}) and the number-average molecular weights (Mₙ) of the copolymers (polymeric additives b)) were determined by gel permeation chromatography (GPC) using poly(methyl-methacrylate) calibration standards according to DIN 55672-1 using the following measurement conditions:
*Column:* the column set consists of a precolumn and 5 SDV columns as disclosed in Table 1:

**Table 1**

| No. | Type | Dimension |
|---|---|---|
| Precolumn | SDV 10µ | 8 X 50 mm |
| Column 1 | SDV LXL 10µ | 8 X 300 mm |
| Column 2 | SDV LinL 10µ | 8 X 300 mm |
| Column 3 | SDV 100Å 10µ | 8 X 300 mm |
| Column 4 | SDV 100Å 10µ | 8 X 300 mm |
| Column 5 | KF-800D | 8 X 100 mm |

*Instruments:* Agilent 1100 Series Pump; PSS SECcurity Inline-Degaser; Agilent 1260 Series Autosampler; Agilent 1100 Series RI-Detector; Agilent 1260 Series UV-Detector; Techlab column oven;
*Oven temperature:* 35 °C;
*Standards:* poly(methyl-methacrylate) (so called PMMA) calibration standards;
*Eluent:* tetrahydrofuran (THF);
*Flow rate: 1* mL/min;
*Injected volume:* 100 µL;
*Detection:* RI at a temperature of 35 °C and UV at a wavelength of 239 nm.

Viscosity was measured using a Discovery HR20 TA instruments rheometer using a 2° cone and Peltier plate geometry. The shear rate was 10x1/s (or s⁻¹). The temperature ramp was 1°C per minute.

Wax content was measured using a Differential Scanning Calorimeter from TA Instruments and analysis via TRIOS software.

Determination of wax species was carried out using an Agilent 6890 series High Temperature Gas Chromatograph.

Pour points were measured according to ASTM D97 in 1 °C steps. The test involves cooling the pyrolysis oil composition at a defined cooling rate and measuring the temperature at which the composition can no longer be poured from a vessel.

### Preparation of the polymeric additives

The polymeric additives OMAC1, OMAC2, OMAC3, OMAC5, and OMAC6 were prepared according to Example 1 (Step 1 and Step 2b) in US10,738,138, using the weight ratios of monomers as shown in Table 2 below.

The polymeric additive OMAC4 was prepared according to Example 1 (Step 1 and Step 2a) in US10,738,138, using the weight ratios of monomers as shown in Table 2.

After polymerization, the solvent is not removed and therefore the resulting polymer is mixed with the oil of polymerization. The polymer content of the polymeric additive is provided in Table 2 for the reproducibility of examples.

### Untreated pyrolysis oils:

Table 3 below shows the characteristics of some untreated pyrolysis oils, wherein the pyrolysis oils A, B, D and G are polyolefin pyrolysis oils produced from the pyrolysis of polyolefins which include high-density polyethylene, low-density polyethylene and polypropylene.

**Table 3: Characteristics of untreated plastic pyrolysis oil (namely, before addition of a polymeric additive of the present invention or a comparative polymeric additive)**

| Property | | **Pyrolysis Oil A** | **Pyrolysis Oil B** | **Pyrolysis Oil D** | **Pyrolysis Oil G** |
|---|---|---|---|---|---|
| Pour Point | [°C] | 51 | 0 | 18 | 51 |
| Wax Appearance Temperature | [°C] | 59 | 48 | 55 | 47 |
| Wax Disappearance Temperature | [°C] | 71 | 53 | 65 | 57 |
| C₁₂-C₁₅ n-hydrocarbons | [wt%] | 12.2 | 0.4 | 0.8 | 1.2 |
| C₁₆-C₁₉ n-paraffins | [wt%] | 1.6 | 0.9 | 1.5 | 1.1 |
| C₂₀-C₂₉ n-paraffins | [wt%] | 9.1 | 0.4 | 2 | 1.7 |
| C₃₀-C₃₉ n-paraffins | [wt%] | 3.6 | 0.2 | 3.7 | 0.6 |
| >C₃₉ n-paraffins | [wt%] | 0.5 | 0 | 2.2 | 0.05 |
| Total C16 or greater n-paraffins | [wt%] | 14.8 | 1.5 | 9.4 | 3.45 |

### Preparation of compositions according to the invention

Examples 1, Example 8, Example 15, and Example 22 are plastic pyrolysis oils before the addition of any polymeric additive according to the invention (untreated pyrolysis oil).

Example 2 was prepared by adding 0.1 g of OMAC1 to 99.9 g of Pyrolysis Oil A. The two components were mixed using an overhead stirrer for 30 minutes while being heated on a hot plate set to 65 °C.

The other composition examples 3-7, 9-14, 16-21, and 23-28 and were prepared in a similar manner as Example 2 using the t polymeric additives and amount indicated in Tables 4-7 below.

**Table 4: Comparative pyrolysis oil compositions compared to the untreated Pyrolysis oil A**

| **Example #** | | **1** | **2** | **3** | **4** | **5** | **6** | **7** |
|---|---|---|---|---|---|---|---|---|
| **Polymer** | | none | OMAC1 | OMAC2 | OMAC3 | OMAC4 | OMAC5 | OMAC6 |
| **Polymer amount** | [g] | 0 | 0.1 | 0.1 | 0.1 | 0.1 | 0.1 | 0.1 |
| **Pyrolysis Oil A amount** | [g] | 100 | 99.9 | 99.9 | 99.9 | 99.9 | 99.9 | 99.9 |
| **PP** | [°C] | 51 | 42 | 40 | 45 | 43 | 45 | 44 |
| **PP Reduction** | [°C] | n/a | 9 | 11 | 6 | 8 | 6 | 7 |
| **Viscosity, 40°C** | [cP] | 925 | 976 | 2412 | 3054 | 5988 | 3035 | 985 |
| **Viscosity Reduction , 40°C** | [%] | n/a | -6 | -161 | -230 | -547 | -228 | -6 |

| | | | | | | | | |
|---|---|---|---|---|---|---|---|---|
| n/a: not applicable (baseline) n.m.: not measured | | | | | | | | |

**Table 5: Pyrolysis oil compositions according to invention compared to the untreated Pyrolysis oil B**

| **Example #** | | **8** | **9** | **10** | **11** | **12** | **13** | **14** |
|---|---|---|---|---|---|---|---|---|
| **Polymer** | | none | OMAC1 | OMAC2 | OMAC3 | OMAC4 | OMAC5 | OMAC6 |
| **Polymer amount** | [g] | 0 | 0.1 | 0.1 | 0.1 | 0.1 | 0.1 | 0.1 |
| **Pyrolysis Oil B amount** | [g] | 100 | 99.9 | 99.9 | 99.9 | 99.9 | 99.9 | 99.9 |
| **PP** | [°C] | 0 | -45 | -39 | -42 | -45 | -48 | -48 |
| **PP Reduction** | [°C] | n/a | 45 | 39 | 42 | 45 | 48 | 48 |
| **Viscosity, - 10°C** | [cP] | 6370 | 4537 | 3250 | 4107 | 4992 | 1453 | 2426 |
| **Viscosity Reduction, - 10°C** | [%] | n/a | 29 | 49 | 36 | 22 | 77 | 62 |

| | | | | | | | | |
|---|---|---|---|---|---|---|---|---|
| n/a: not applicable (baseline) n.m.: not measured | | | | | | | | |

**Table 6: Pyrolysis oil compositions according to invention compared to the untreated Pyrolysis oil D**

| **Example #** | | **15** | **16** | **17** | **18** | **19** | **20** | **21** |
|---|---|---|---|---|---|---|---|---|
| **Polymer** | | none | OMAC1 | OMAC2 | OMAC3 | OMAC4 | OMAC5 | OMAC6 |
| **Polymer amount** | [g] | 0 | 0.1 | 0.1 | 0.1 | 0.1 | 0.1 | 0.1 |
| **Pyrolysis Oil D amount** | [g] | 100 | 99.9 | 99.9 | 99.9 | 99.9 | 99.9 | 99.9 |
| **PP** | [°C] | 18 | 6 | 9 | 12 | 6 | 3 | 3 |
| **PP Reduction** | [°C] | n/a | 12 | 9 | 6 | 12 | 15 | 15 |
| **Viscosity, 10°C** | [cP] | 145981 | 33420 | 6122 | 1789 | 14235 | 18432 | 31143 |
| **Viscosity Reduction, 10°C** | [%] | n/a | 77 | 96 | 99 | 90 | 87 | 79 |

| | | | | | | | | |
|---|---|---|---|---|---|---|---|---|
| n/a: not applicable (baseline) n.m.: not measured | | | | | | | | |

**Table 7: Pyrolysis oil compositions according to invention compared to the untreated Pyrolysis oil G**

| **Example #** | | **22** | **23** | **24** | **25** | **26** | **27** | **28** |
|---|---|---|---|---|---|---|---|---|
| **Polymer** | | none | OMAC1 | OMAC2 | OMAC3 | OMAC4 | OMAC5 | OMAC6 |
| **Polymer amount** | [g] | 0 | 0.1 | 0.1 | 0.1 | 0.1 | 0.1 | 0.1 |
| **Pyrolysis Oil G amount** | [g] | 100 | 99.9 | 99.9 | 99.9 | 99.9 | 99.9 | 99.9 |
| **PP** | [°C] | 51 | 15 | 42 | 42 | 45 | 45 | 42 |
| **PP Reduction** | [°C] | n/a | 36 | 9 | 9 | 6 | 6 | 9 |
| **Viscosity, 40°C** | [cP] | 59973 | 922 | 967 | 845 | 2404 | 3208 | 770 |
| **Viscosity Reduction, 40°C** | [%] | n/a | 98.5 | 98.4 | 98.6 | 96 | 94.7 | 98.7 |

| | | | | | | | | |
|---|---|---|---|---|---|---|---|---|
| n/a: not applicable (baseline) n.m.: not measured | | | | | | | | |

### Results

Table 4 shows that addition of OMAC copolymers into a pyrolysis oil with a content of more than 14 wt% of C₁₆ or greater n-paraffins, an undesirable increase in viscosity is observed. Examples 2-7 show that the viscosity of Pyrolysis Oil A, treated with the OMAC copolymers, disadvantageously increases significantly from 6 to 547 %. This large increase in viscosity would make the oil much more difficult to handle and transport.

In contrast, when the OMAC polymers of the invention are combined with a pyrolysis oil having a content of 12 wt% or less of C₁₆ or greater n-paraffins, a reduction in viscosity, as well as a reduction in pour point are advantageously both achieved when compared to the same pyrolysis oil with no polymeric additive. This is the most desirable outcome where the treated pyrolysis oil will flow at a lower temperature (reduced pour point) and have a lower viscosity for improved handling properties.

Similarly, Examples 9-14 demonstrate how the OMAC copolymers achieve this reduction in pour point and viscosity when added to Pyrolysis Oil B. Compared to the untreated oil (Example 8), Examples 9-14 have a 39-48 °C lower pour point and 29-77 % reduction in viscosity.

The same is true for Examples 16-21, which demonstrate how the OMAC copolymers achieve this reduction in pour point and viscosity when added to Pyrolysis Oil D. Compared to the untreated oil (Example 15), Examples 16-21 have a 6-15 °C lower pour point and 77-99 % reduction in viscosity.

Examples 23-28 demonstrate how the OMAC copolymers achieve this reduction in pour point and viscosity when added to Pyrolysis Oil G. Compared to the untreated oil (Example 22), Examples 23-28 have a 6-36 °C lower pour point and >95 % reduction in viscosity.

It has been shown that the OMAC copolymers are specifically most effective in the treatment of plastic pyrolysis oils from a plastic pyrolysis process having a content of 12 wt% or less of C₁₆ or greater n-paraffins. The experimental data demonstrate how the addition of OMAC copolymers to plastic pyrolysis oils having a content of 12 wt% or less of C₁₆ or greater n-paraffins advantageously keep them liquid, improving the transport and storage of these oils before the cracking process, by effectively lowering their pour point and/or lowering their viscosity.

## Claims

1. A composition comprising a plastic pyrolysis oil a) and a polymeric additive b), wherein the polymeric additive b) is a copolymer P) prepared by polymerizing a monomer composition comprising
i) 10 to 70 % by weight of monomers selected from alkyl maleate compound of Formula (I), maleimide compound of Formula (II) or a mixture thereof, based on the total weight of the copolymer, wherein R" in Formula (I) and Formula (II) is a linear or branched alkyl group having from 10 to 40 carbon atoms, preferably from 10 to 30 carbon atoms, more preferably from 12 to 30 carbon atoms, even more preferably from 18 to 22 carbon atoms;
and
ii) 30 to 90 % by weight of a non-functionalized alpha-olefin of Formula (III) or a mixture thereof, based on the total weight of the copolymer, wherein R₂ is a linear alkyl group having from 8 to 40 carbon atoms, preferably from 10 to 40 carbon atoms, more preferably from 15 to 35 carbon atoms, even more preferably from 20 to 32 carbon atoms, and
wherein the plastic pyrolysis oil a) comprises 12 % by weight or less of n-paraffin waxes with C₁₆ or longer carbon chains, based on the total weight of the plastic pyrolysis oil a).

2. The composition according to claim 1, wherein the polymeric additive b) is a copolymer P) prepared by polymerizing a monomer composition comprising
i) 10 to 70 % of alkyl maleate compound of Formula (I), based on the total weight of the copolymer, and
ii) 30 to 90 % by weight of the non-functionalized alpha-olefin of Formula (III),
based on the total weight of the copolymer P).

3. The composition according to claim 1 or 2, wherein the monomer composition of copolymer P) comprises 20 to 50 % by weight, preferably 25 to 40 % by weight, of alkyl maleate compound of Formula (I), based on the total weight of the copolymer P).

4. The composition according to any one of the preceding claims, wherein the monomer composition of copolymer P) comprises from 50 to 80 % by weight, preferably from 60 to 75 % by weight, of non-functionalized alpha-olefin of Formula (III), based on the total weight of the copolymer P).

5. The composition according to any one of the preceding claims, wherein the copolymer P) is selected from the group consisting of a polymer prepared by polymerizing a monomer composition comprising C₁₈-C₂₂ alkyl maleate and C₂₀-C₃₂ non-functionalized alpha-olefin, or a polymer prepared by polymerizing a monomer composition comprising C₁₈-C₂₂ alkyl maleate and C₂₀-C₂₄ non-functionalized alpha-olefin, or a polymer prepared by polymerizing a monomer composition comprising C₁₈-C₂₂ alkyl maleate and C₁₀-C₁₈ non-functionalized alpha-olefin, or a mixture thereof.

6. The composition according to any one of the preceding claims, wherein the monomer composition to prepare the copolymer P) further comprises monomers iii) selected from the group consisting of:
hydroxyalkyl (meth)acrylates, preferably hydroxyalkyl (meth)acrylates selected from 3-hydroxypropyl (meth)acrylate, 3,4-dihydroxybutyl (meth)acrylate, 2-hydroxyethyl (meth)acrylate, 2 hydroxypropyl (meth)acrylate, 2,5-dimethyl-1,6-hexanediol (meth)acrylate, 1,10 decanediol (meth)acrylate;
aminoalkyl (meth)acrylates and aminoalkyl (meth)acrylamides, preferably aminoalkyl (meth)acrylates and aminoalkyl (meth)acrylamides selected from N-(3-dimethyl-aminopropyl)methacrylamide, 3-diethylaminopentyl (meth)acrylate, 3-dibutyl-aminohexadecyl (meth)acrylate;
nitriles of (meth)acrylic acid and other nitrogen-containing (meth)acrylates, preferably nitriles of (meth)acrylic acid and other nitrogen-containing (meth)acrylates selected from N-(methacryloyloxyethyl)diisobutylketimine, N-(methacryloyloxyethyl)dihexadecyl-ketimine, (meth)acryloylamidoacetonitrile, 2-methacryloyloxyethylmethylcyanamide, cyanomethyl (meth)acrylate;
aryl (meth)acrylates like benzyl (meth)acrylate or phenyl (meth)acrylate, where the acryl residue in each case can be unsubstituted or substituted up to four times;
carbonyl-containing (meth)acrylates, preferably carbonyl-containing (meth)acrylates selected from 2-carboxyethyl (meth)acrylate, carboxymethyl (meth)acrylate, N-methyacryloyloxy)-formamide, acetonyl (meth)acrylate, N-methacryloyl-2 pyrrolidinone, N-(2-methyacryloxyoxyethyl)-2-pyrrolidinone, N-(3-methacryloyloxy-propyl)-2-pyrrolidinone, N-(2-methyacryloyloxypentadecyl(-2-pyrrolidinone, N-(3 methacryloyloxyheptadecyl-2-pyrrolidinone;
(meth)acrylates of ether alcohols, preferably (meth)acrylates of ether alcohols selected from tetrahydrofurfuryl (meth)acrylate, methoxyethoxyethyl (meth)acrylate, 1-butoxypropyl (meth)acrylate, cyclohexyloxyethyl (meth)acrylate, propoxyethoxyethyl (meth)acrylate, benzyloxyethyl (meth)acrylate, furfuryl (meth)acrylate, 2-butoxyethyl (meth)acrylate, 2-ethoxy-2-ethoxyethyl (meth)acrylate, 2-methoxy-2-ethoxypropyl (meth)acrylate, ethoxylated (meth)acrylates, 1-ethoxybutyl (meth)acrylate, methoxyethyl (meth)acrylate, 2-ethoxy-2-ethoxy-2-ethoxyethyl (meth)acrylate, esters of (meth)acrylic acid and methoxy polyethylene glycols;
(meth)acrylates of halogenated alcohols, preferably (meth)acrylates of halogenated alcohols selected from 2,3-dibromopropyl (meth)acrylate, 4 bromophenyl (meth)acrylate, 1,3-dichloro-2-propyl (meth)acrylate, 2-bromoethyl (meth)acrylate, 2-iodoethyl (meth)acrylate, chloromethyl (meth)acrylate;
oxiranyl (meth)acrylate, preferably oxiranyl (meth)acrylate selected from 2, 3-epoxybutyl (meth)acrylate, 3,4-epoxybutyl (meth)acrylate, 10,11-epoxyundecyl (meth)acrylate, 2,3-epoxycyclohexyl (meth)acrylate, oxiranyl (meth)acrylates such as 10,11-epoxyhexadecyl (meth)acrylate, glycidyl (meth)acrylate;
phosphorus-, boron- and/or silicon-containing (meth)acrylates, preferably phosphorus-, boron- and/or silicon-containing (meth)acrylates selected from 2-(dimethyl-phosphato)propyl (meth)acrylate, 2-(ethylphosphito)propyl (meth)acrylate, 2 dimethylphosphinomethyl (meth)acrylate, dimethylphosphonoethyl (meth)acrylate, diethylmethacryloyl phosphonate, dipropylmethacryloyl phosphate, 2 (dibutylphosphono)ethyl (meth)acrylate, 2,3-butylenemethacryloylethyl borate, methyldiethoxymethacryloylethoxysiliane, diethylphosphatoethyl (meth)acrylate;
sulfur-containing (meth)acrylates, preferably sulfur-containing (meth)acrylates selected from ethylsulfinylethyl (meth)acrylate, 4-thio-cyanatobutyl (meth)acrylate, ethylsulfonylethyl (meth)acrylate, thiocyanatomethyl (meth)acrylate, methylsulfinylmethyl (meth)acrylate, bis(methacryloyloxyethyl) sulfide;
heterocyclic (meth)acrylates, preferably heterocyclic (meth)acrylates selected from 2-(1-imidazolyl)ethyl (meth)acrylate, oxazolidinylethyl (meth)acrylate, N-methacryloylmorpholine and 2-(4-morpholinyl)ethyl (meth)acrylate;
maleic acid and maleic acid derivatives, preferably mono- and diesters of maleic acid, maleic anhydride, methylmaleic anhydride, maleinimide, methylmaleinimide;
fumaric acid and fumaric acid derivatives, preferably mono- and diesters of fumaric acid;
vinyl halides, preferably vinyl halides selected from vinyl chloride, vinyl fluoride, vinylidene chloride and vinylidene fluoride;
vinyl esters, preferably vinyl acetate;
vinyl monomers containing aromatic groups, preferably vinyl monomers containing aromatic groups selected from styrene, substituted styrenes with an alkyl substituent in the side chain, such as alpha-methylstyrene and alpha-ethylstyrene, substituted styrenes with an alkyl substituent on the ring such as vinyltoluene and p-methylstyrene, halogenated styrenes such as monochlorostyrenes, dichlorostyrenes, tribromostyrenes and tetrabromostyrenes;
heterocyclic vinyl compounds, preferably heterocyclic vinyl compounds selected from 2-vinylpyridine, 3-vinylpyridine, 2-methyl-5-vinylpyridine, 3-ethyl-4-vinylpyridine, 2,3-dimethyl-5-vinylpyridine, vinylpyrimidine, vinylpiperidine, 9-vinylcarbazole, 3-vinylcarbazole, 4-vinylcarbazole, 1-vinylimidazole, 2-methyl-1-vinylimidazole, N-vinylpyrrolidone, 2-vinylpyrrolidone, N-vinylpyrrolidine, 3-vinylpyrrolidine, N-vinylcaprolactam, N-vinylbutyrolactam, vinyloxolane, vinylfuran, vinylthiophene, vinylthiolane, vinylthiazoles and hydrogenated vinylthiazoles, vinyloxazoles and hydrogenated vinyloxazoles;
vinyl and isoprenyl ethers;
methacrylic acid and acrylic acid, or a mixture thereof.

7. The composition according to any one of the preceding claims, wherein the composition comprises from 0.001 to 1 % by weight, preferably from 0.005 to 0.8 % by weight, more preferably from 0.005 to 0.5 % by weight of the polymeric additive b), based on the total weight of the composition.

8. The composition according to any one of the preceding claims, wherein the copolymer P) has a weight-average molecular weight is from 8,000 to 600,000 g/mol, preferably from 8,000 to 300,000 g/mol even more preferably from 8,000 to 100,000 g/mol and most preferably from 10,000 to 50,000 g/mol, determined by gel permeation chromatography using poly(methyl-methacrylate) calibration standards according to DIN 55672-1.

9. The composition according to any one of the preceding claims, wherein the plastic pyrolysis oil a) is a plastic pyrolysis oil and/or a plastic waste pyrolysis oil, wherein the plastic and plastic waste are selected from polyolefins, polyethylene terephthalate, polyvinyl chloride, polystyrene, or a mixture thereof.

10. The composition according to claim 9, wherein the plastic pyrolysis oil a) comprises from 0 % to 12 % of C₁₆ to C₁₉ n-paraffin waxes, from 0 % to 12 % of C₂₀ to C₂₉ n-paraffin waxes, from 0 % to 12 % of C₃₀ to C₃₉ n-paraffin waxes, and from 0 % to 12 % of n-paraffin waxes with C₄₀ or longer carbon chains, wherein the total wax content of n-paraffin waxes with C₁₆ or longer carbon chains sums up to 12 % by weight or less, based on the total weight of the plastic pyrolysis oil.

11. The composition according to any one of the preceding claims, wherein the composition further comprises an additive c), wherein the additive c) is any of the group comprising scale inhibitors, corrosion inhibitors, oxygen scavengers, biocides, emulsion breakers, antifoam agents, drag reducing agents, hydrate inhibitors, paraffin dispersants, asphaltene control agents, a pour point depressant other than copolymer P), or a mixture thereof.

12. The composition according to any one of the preceding claims, wherein the polymeric additive b) reduces the pour point of the pyrolysis oil a) by at least 1 °C, or wherein the polymeric additive b) reduces the viscosity of the pyrolysis oil a) by at least 10% at a temperature from -20 °C to +80 °C, or both.

13. A method of manufacturing the composition as defined in any one of claims 1 to 12 comprising the steps of:
providing a plastic feedstock;
pyrolyzing the plastic feedstock to generate the plastic pyrolysis oil a);
preparing the polymeric additive b) and
adding the polymeric additive b) to the plastic pyrolysis oil a).

14. Use of a polymeric additive b) as defined in any one of claims 1 to 12 to reduce the pour point of a plastic pyrolysis oil a) or to reduce the viscosity of the plastic pyrolysis oil a), or both.

15. A method of transporting or storing a plastic pyrolysis oil a) comprising the step of adding a polymeric additive b) to the plastic pyrolysis oil a), to form a composition as defined in any one of claims 1 to 12.

## Patentansprüche

1. Zusammensetzung umfassend ein Kunststoffpyrolyseöl a) und einen polymeren Zusatzstoff b), wobei der polymere Zusatzstoff b) ein Copolymer P) ist, das durch Polymerisation einer Monomerzusammensetzung hergestellt ist, die umfasst
i) 10 bis 70 Gew.-% Monomere ausgewählt aus Alkylmaleatverbindung der Formel (I), Maleimidverbindung der Formel (II) oder einem Gemisch davon, bezogen auf das Gesamtgewicht des Copolymers, wobei R" in Formel (I) und Formel (II) eine lineare oder verzweigte Alkylgruppe mit von 10 bis 40 Kohlenstoffatomen, vorzugsweise von 10 bis 30 Kohlenstoffatomen, bevorzugter von 12 bis 30 Kohlenstoffatomen, noch bevorzugter von 18 bis 22 Kohlenstoffatomen, ist;
und
ii) 30 bis 90 Gew.-% an einem nichtfunktionalisierten alpha-Olefin der Formel (III) oder einem Gemisch davon, bezogen auf das Gesamtgewicht des Copolymers,
wobei R₂ eine lineare Alkylgruppe mit von 8 bis 40 Kohlenstoffatomen, vorzugsweise von 10 bis 40 Kohlenstoffatomen, bevorzugter von 15 bis 35 Kohlenstoffatomen, noch bevorzugter von 20 bis 32 Kohlenstoffatomen, ist, und
wobei das Kunststoffpyrolyseöl a) 12 Gew.-% oder weniger n-Paraffinwachse mit C₁₆- oder längeren Kohlenstoffketten, bezogen auf das Gesamtgewicht des Kunststoffpyrolyseöls a), umfasst.

2. Zusammensetzung nach Anspruch 1, wobei der polymere Zusatzstoff b) ein Copolymer P) ist, hergestellt durch Polymerisation einer Monomerzusammensetzung umfassend
i) 10 bis 70 Gew.-% Alkylmaleatverbindung der Formel (I) bezogen auf das Gesamtgewicht des Copolymers und
ii) 30 bis 90 Gew.-% an dem nichtfunktionalisierten alpha-Olefin der Formel (III) bezogen auf das Gesamtgewicht des Copolymers P).

3. Zusammensetzung nach Anspruch 1 oder 2, wobei die Monomerzusammensetzung des Copolymers P) 20 bis 50 Gew.-%, vorzugsweise 25 bis 40 Gew.-%, Alkylmaleatverbindung der Formel (I), bezogen auf das Gesamtgewicht des Copolymers P), umfasst.

4. Zusammensetzung nach einem der vorstehenden Ansprüche, wobei die Monomerzusammensetzung des Copolymers P) von 50 bis 80 Gew.-%, vorzugsweise von 60 bis 75 Gew.-%, an dem nichtfunktionalisierten alpha-Olefin der Formel (III) bezogen auf das Gesamtgewicht des Copolymers P) umfasst.

5. Zusammensetzung nach einem der vorstehenden Ansprüche, wobei das Copolymer P) ausgewählt ist aus der Gruppe bestehend aus einem Polymer, hergestellt durch Polymerisation einer Monomerzusammensetzung, die C₁₈-C₂₂-Alkylmaleat und nichtfunktionalisiertes C₂₀-C₃₂-alpha-Olefin umfasst, oder ein Polymer, hergestellt durch Polymerisation einer Monomerzusammensetzung, die C₁₈-C₂₂-Alkylmaleat und nichtfunktionalisiertes C₂₀-C₂₄-alpha-Olefin umfasst, oder ein Polymer, hergestellt durch Polymerisation einer Monomerzusammensetzung, die C₁₈-C₂₂-Alkylmaleat und nichtfunktionalisiertes C₁₀-C₁₈-alpha-Olefin umfasst, oder ein Gemisch davon.

6. Zusammensetzung nach einem der vorstehenden Ansprüche, wobei die Monomerzusammensetzung zur Herstellung des Copolymers P) ferner Monomere iii) umfasst, ausgewählt aus der Gruppe bestehend aus:
Hydroxyalkyl(meth)acrylaten, vorzugsweise Hydroxyalkyl(meth)acrylaten ausgewählt aus 3-Hydroxypropyl(meth)acrylat, 3,4-Dihydroxybutyl(meth)acrylat, 2-Hydroxyethyl(meth)acrylat, 2-Hydroxypropyl(meth)acrylat, 2,5-Dimethyl-1,6-hexandiol(meth)acrylat, 1,10-Decandiol(meth)acrylat;
Aminoalkyl(meth)acrylaten und Aminoalkyl(meth)acrylamiden, vorzugsweise Aminoalkyl(meth)acrylaten und Aminoalkyl(meth)acrylamiden ausgewählt aus N-(3-Dimethylaminopropyl)methacrylamid, 3-Diethylaminopentyl(meth)acrylat, 3-Dibutylaminohacrylat(meth)acrylat;
Nitrilen von (Meth)acrylsäure und anderen stickstoffhaltigen (Meth)acrylaten, vorzugsweise Nitrilen von (Meth)acrylsäure und anderen stickstoffhaltigen (Meth)acrylaten ausgewählt aus N-(Methacryloyloxyethyl)diisobutylketimin, N-(Methacryloyloxyethyl)dihexadecylketimin, (Meth)acryloylamidoacetonitril, 2-Methacryloyloxyethylmethylcyanamid,
Cyanomethyl(meth)acrylat;
Aryl(meth)acrylaten wie Benzyl(meth)acrylat oder Phenyl(meth)acrylat, wobei der Acrylrest in jedem Fall unsubstituiert oder bis zu viermal substituiert sein kann;
carbonylhaltigen (Meth)acrylaten, vorzugsweise carbonylhaltigen (Meth)acrylaten ausgewählt aus 2-Carboxyethyl(meth)acrylat, Carboxymethyl(meth)acrylat, N-(Methyacryloyloxy)formamid, Acetonyl(meth)acrylat, N-Methacryloyl-2-pyrrolidinon, N-(2-Methyacryloxyoxyethyl)-2-pyrrolidinon, N-(3-Methacryloyloxypropyl)-2-pyrrolidinon, N-(2-Methyacryloyloxypentadecyl(-2-pyrrolidinon, N-(3-Methacryloyloxyheptadecyl-2-pyrrolidinon;
(Meth)acrylaten von Etheralkoholen, vorzugsweise (Meth)acrylaten von Etheralkoholen ausgewählt aus Tetrahydrofuryl(meth)acrylat, Methoxyethoxyethyl(meth)acrylat, 1-Butoxypropyl(meth)acrylat, Cyclohexyloxyethyl(meth)acrylat, Propoxyethoxyethyl(meth)acrylat, Benzyloxyethyl(meth)acrylat, Furfuryl(meth)acrylat, 2-Butoxyethyl(meth)acrylat, 2-Ethoxy-2-ethoxyethyl(meth)acrylat, 2-Methoxy-2-ethoxypropyl(meth)acrylat, ethoxylierten (Meth)acrylaten, 1-Ethoxybutyl(meth)acrylat, Methoxyethyl(meth)acrylat, 2-Ethoxy-2-ethoxy-2-ethoxyethyl(meth)acrylat, Estern von (Meth)acrylsäure und Methoxypolyethylenglycolen;
(Meth)acrylaten von halogenierten Alkoholen, vorzugsweise (Meth)acrylaten von halogenierten Alkoholen ausgewählt aus 2,3-Dibrompropyl(meth)acrylat, 4-Bromophenyl(meth)acrylat, 1,3-Dichlor-2-propyl(meth)acrylat, 2-Bromethyl(meth)acrylat, 2-Iodethyl(meth)acrylat, Chlormethyl(meth)acrylat;
Oxiranyl(meth)acrylaten, vorzugsweise Oxiranyl(meth)acrylaten ausgewählt aus 2,3-Epoxybutyl(meth)acrylat, 3,4-Epoxybutyl(meth)acrylat, 10,11-Epoxyundecyl(meth)acrylat, 2,3-Epoxycyclohexyl(meth)acrylat, Oxiranyl(meth)acrylaten, wie z.B. wie 10,11-Epoxyhexadecyl(meth)acrylat, Glycidyl(meth)acrylat;
phosphor-, bor- und/oder siliciumhaltigen (Meth)acrylaten, vorzugsweise phosphor-, bor- und/oder siliciumhaltigen (Meth)acrylaten ausgewählt aus 2-(Dimethylphosphato)propyl(meth)acrylat, 2-(Ethylphosphito)propyl(meth)acrylat, 2-Dimethylphosphinomethyl(meth)acrylat, Dimethylphosphonoethyl(meth)acrylat, Diethylmethacryloylphosphonat, Dipropylmethacryloylphosphat, 2-(Dibutylphosphono)ethyl(meth)acrylat, 2,3-Butylenmethacryloylethylborat, Methyldiethoxymethacryloylethoxysilian, Diethylphosphatoethyl(meth)acrylat;
schwefelhaltigen (Meth)acrylaten, vorzugsweise schwefelhaltigen (Meth)acrylaten ausgewählt aus Ethylsulfinylethyl(meth)acrylat, 4-Thio-cyanatobutyl(meth)acrylat, Ethylsulfonylethyl(meth)acrylat, Thiocyanatomethyl(meth)acrylat, Methylsulfinylmethyl(meth)acrylat) , Bis(methacryloyloxyethyl)sulfid;
heterocyclischen (Meth)acrylaten, vorzugsweise heterocyclischen (Meth)acrylaten ausgewählt aus 2-(1-Imidazolyl)ethyl (meth)acrylat, Oxazolidinylethyl(meth)acrylat, N-Methacryloylmorpholin und 2-(4-Morpholinyl)ethyl(meth)acrylat;
Maleinsäure und Maleinsäurederivaten, vorzugsweise Mono- und Diestern von Maleinsäure, Maleinsäureanhydrid, Methylmaleinsäureanhydrid, Maleinimid, Methylmaleinimid; Fumarsäure und Fumarsäurederivaten, vorzugsweise Mono- und Diestern von Fumarsäure;
Vinylhalogeniden, vorzugsweise Vinylhalogeniden ausgewählt aus Vinylchlorid, Vinylfluorid, Vinylidenchlorid und Vinylidenfluorid;
Vinylestern, vorzugsweise Vinylacetat;
Vinylmonomeren, die aromatische Gruppen enthalten, vorzugsweise Vinylmonomeren, die aromatische Gruppen enthalten, ausgewählt aus Styrol, substituierten Styrolen mit einem Alkylsubstituenten in der Seitenkette, wie z.B. alpha-Methylstyrol und alpha-Ethylstyrol, substituierten Styrolen mit einem Alkylsubstituenten an dem Ring, wie z.B. Vinyltoluol und p-Methylstyrol, halogeniertem Styrol, Dichlorstyrol, Trimostyrol und Styrol;
heterocyclischen Vinylverbindungen, vorzugsweise heterocyclischen Vinylverbindungen ausgewählt aus 2-Vinylpyridin, 3-Vinylpyridin, 2-Methyl-5-vinylpyridin, 3-Ethyl-4-vinylpyridin, 2,3-Dimethyl-5-vinylpyridin, Vinylpyrimidin, Vinylpiperidin, 9-Vinylcarbazol, 3-Vinylcarbazol, 4-Vinylcarbazol, 1-Vinylimidazol, 2-Methyl-1-vinylimidazol, N-Vinylpyrrolidon, 2-Vinylpyrrolidon, N-Vinylpyrrolidin, 3-Vinylpyrrolidin, N-Vinylcaprolactam, N-Vinylbutyrolactam, Vinyloxolan, Vinylfuran, Vinylthiophen, Vinylthiolan, Vinylthiazolen und hydrierten Vinylthiazolen, Vinyloxazolen und hydrierten Vinyloxazolen;
Vinyl- und Isoprenylethern,
Methacrylsäure und Acrylsäure oder einem Gemisch davon.

7. Zusammensetzung nach einem der vorstehenden Ansprüche, wobei die Zusammensetzung von 0,001 bis 1 Gew.-%, vorzugsweise von 0,005 bis 0,8 Gew.-%, bevorzugter von 0,005 bis 0,5 Gew.-%, an dem polymeren Zusatzstoff b), bezogen auf das Gesamtgewicht der Zusammensetzung, umfasst.

8. Zusammensetzung nach einem der vorstehenden Ansprüche, wobei das Copolymer P) ein gewichtsgemitteltes Molekulargewicht von 8.000 bis 600.000 g/mol, vorzugsweise von 8.000 bis 300.000 g/mol, bevorzugter von 8.000 bis 100.000 g/mol und höchst bevorzugt von 10.000 bis 50.000 g/mol aufweist, bestimmt durch Gelpermeationschromatographie unter Verwendung von Poly(methylmethacrylat)-Kalibrierstandards nach DIN 55672-1.

9. Zusammensetzung nach einem der vorstehenden Ansprüche, wobei das Kunststoffpyrolyseöl a) ein Kunststoffpyrolyseöl und/oder ein Kunststoffabfallpyrolyseöl ist, wobei der Kunststoff und der Kunststoffabfall ausgewählt sind aus Polyolefinen, Polyethylenterephthalat, Polyvinylchlorid, Polystyrol oder einem Gemisch davon.

10. Zusammensetzung nach Anspruch 9, wobei das Kunststoffpyrolyseöl a) von 0 % bis 12 % an C₁₆- bis C₁₉-n-Paraffinwachsen, von 0 % bis 12 % an C₂₀- bis C₂₉-n-Paraffinwachsen, von 0 % bis 12 % an C₃₀- bis C₃₉-n-Paraffinwachsen und von 0 bis 12 Gew.-% an n-Paraffinwachsen mit C₄₀ oder längeren Kohlenstoffketten umfasst, wobei der Gesamtwachsgehalt von n-Paraffinwachsen mit C₁₆ oder längeren Kohlenstoffketten bis zu 12 Gew.-% oder weniger beträgt, bezogen auf das Gesamtgewicht des Kunststoffpyrolyseöls.

11. Zusammensetzung nach einem der vorstehenden Ansprüche, wobei die Zusammensetzung ferner einen Zusatzstoff c) umfasst, wobei der Zusatzstoff c) einer aus der Gruppe umfassend Ablagerungshemmer, Korrosionshemmer, Sauerstofffänger, Biozide, Emulsionsbrecher, Antischaummittel, Widerstandsverringerungsmittel, Hydratinhibitoren, Paraffindispergiermittel, Asphaltenbekämpfungsmittel, Pourpoint-Senker, die von Copolymer P) verschieden sind, oder ein Gemisch davon ist.

12. Zusammensetzung nach einem der vorstehenden Ansprüche, wobei der polymere Zusatzstoff b) den Pourpoint des Pyrolyseöls a) um wenigstens 1 °C senkt oder wobei der polymere Zusatzstoff b) die Viskosität des Pyrolyseöls a) um wenigstens 10 % bei einer Temperatur von -20 °C bis +80 °C senkt, oder beides.

13. Verfahren zur Herstellung der Zusammensetzung nach einem der Ansprüche 1 bis 12, umfassend die Schritte:
Bereitstellen eines Kunststoff-Einsatzmaterials;
Pyrolysieren des Kunststoff-Einsatzmaterials, um das Kunststoffpyrolyseöl a) zu erzeugen;
Herstellen des polymeren Zusatzstoffs b) und
Zugeben des polymeren Zusatzstoffs b) zu dem Pyrolyseöl a).

14. Verwendung eines polymeren Zusatzstoffs b) nach einem der Ansprüche 1 bis 12 zum Senken des Pourpoints eines Kunststoffpyrolyseöls a) oder zum Senken der Viskosität des Kunststoffpyrolyseöls a) oder von beiden.

15. Verfahren zum Befördern oder Lagern eines Kunststoffpyrolyseöls a), umfassend den Schritt des Zugebens eines polymeren Zusatzstoffs b) zu dem Kunststoffpyrolyseöl a), um eine Zusammensetzung nach einem der Ansprüche 1 bis 12 zu bilden.

## Revendications

1. Composition comprenant une huile de pyrolyse de plastique a) et un additif polymérique b), dans laquelle l'additif polymérique b) est un copolymère P) préparé par polymérisation d'une composition de monomères comprenant
i) 10 à 70 % en poids de monomères choisis parmi un composé de maléate d'alkyle de formule (I), un composé de maléimide de formule (II) ou un mélange de ceux-ci, par rapport au poids total du copolymère, dans laquelle R" dans la formule (I) et la formule (II) est un groupe alkyle linéaire ou ramifié ayant de 10 à 40 atomes de carbone, de préférence de 10 à 30 atomes de carbone, plus préférablement de 12 à 30 atomes de carbone, encore plus préférablement de 18 à 22 atomes de carbone ;
et
ii) 30 à 90 % en poids d'une alpha-oléfine non fonctionnalisée de formule (III) ou d'un mélange de celles-ci, par rapport au poids total du copolymère,
dans laquelle R₂ est un groupe alkyle linéaire ayant de 8 à 40 atomes de carbone, de préférence de 10 à 40 atomes de carbone, plus préférentiellement de 15 à 35 atomes de carbone, encore plus préférablement de 20 à 32 atomes de carbone, et
dans laquelle l'huile de pyrolyse de plastique a) contient 12 % en poids ou moins de cires n-paraffiniques avec des chaînes carbonées en C₁₆ ou plus longues, par rapport au poids total de l'huile de pyrolyse de plastique a).

2. Composition selon la revendication 1, dans laquelle l'additif polymérique b) est un copolymère P) préparé par polymérisation d'une composition de monomères comprenant
i) 10 à 70 % de composé de maléate d'alkyle de formule (I), par rapport au poids total du copolymère, et
ii) 30 à 90 % en poids de l'alpha-oléfine non fonctionnalisée de formule (III), par rapport au poids total du copolymère P).

3. Composition selon la revendication 1 ou 2, dans laquelle la composition de monomères du copolymère P) comprend de 20 à 50 % en poids, de préférence de 25 à 40 % en poids, d'un composé de maléate d'alkyle de formule (I), par rapport au poids total du copolymère P).

4. Composition selon l'une quelconque des revendications précédentes, dans laquelle la composition de monomères du copolymère P) comprend de 50 à 80 % en poids, de préférence de 60 à 75 % en poids, d'alpha-oléfine non fonctionnalisée de formule (III), par rapport au poids total du copolymère P).

5. Composition selon l'une quelconque des revendications précédentes, dans laquelle le copolymère P) est choisi dans le groupe constitué par un polymère préparé par polymérisation d'une composition de monomères comprenant un maléate d'alkyle en C₁₈-C₂₂ et une alpha-oléfine non fonctionnalisée en C₂₀-C₃₂, ou un polymère préparé par polymérisation d'une composition de monomères comprenant un maléate d'alkyle en C₁₈-C₂₂ et une alpha-oléfine non fonctionnalisée en C₂₀-C₂₄, ou un polymère préparé par polymérisation d'une composition de monomères comprenant un maléate d'alkyle en C₁₈-C₂₂ et une alpha-oléfine non fonctionnalisée en C₁₀-C₁₈, ou un mélange de ceux-ci.

6. Composition selon l'une quelconque des revendications précédentes, dans laquelle la composition de monomères pour préparer le copolymère P) comprend en outre des monomères iii) choisis dans le groupe constitué par :
(méth)acrylates d'hydroxyalkyle, de préférence (méth)acrylates d'hydroxyalkyle choisis parmi (méth)acrylate de 3-hydroxypropyle, (méth)acrylate de 3,4-dihydroxybutyle, (méth)acrylate de 2-hydroxyéthyle, (méth)acrylate de 2-hydroxypropyle, (méth)acrylate de 2,5-diméthyl-1,6-hexanediol, (méth)acrylate de 1,10-décanediol ;
(méth)acrylates d'aminoalkyle et (méth)acrylamides d'aminoalkyle, de préférence (méth)acrylates d'aminoalkyle et (méth)acrylamides d'aminoalkyle choisis parmi le N-(3-diméthylaminopropyl)méthacrylamide, le (méth)acrylate de 3-diéthylaminopentyle, le (méth)acrylate de 3-dibutylaminohexadécyle ;
nitriles d'acide (méth)acrylique et autres (méth)acrylates contenant de l'azote, de préférence des nitriles d'acide (méth)acrylique et autres (méth)acrylates contenant de l'azote choisis parmi la N-(méthacryloyloxyéthyl)diisobutylcétimine, la N-(méthacryloyloxyéthyl)dihexadécylcétimine, le (méth)acryloylamidoacétonitrile, le 2-méthacryloyloxyéthylméthylcyanamide, le (méth)acrylate de cyanométhyle ;
(méth)acrylates d'aryle comme le (méth)acrylate de benzyle ou le (méth)acrylate de phényle, où le radical acryle en chaque cas peut être non substitué ou substitué jusqu'à quatre fois ;
(méth)acrylates contenant carbonyle, de préférence des (méth)acrylates contenant carbonyle choisis parmi le (méth)acrylate de 2-carboxyéthyle, le (méth)acrylate de carboxyméthyle, le N-méthyacryloyloxy)-formamide, le (méth)acrylate d'acétonyle, la N-méthacryloyl-2 pyrrolidinone, la N-(2-méthyacryloxyoxyéthyl)-2-pyrrolidinone, la N-(3-méthacryloyloxypropyl)-2-pyrrolidinone, la N-(2-méthyacryloyloxypentadécyl (-2-pyrrolidinone, la N-(3 méthacryloyloxyheptadécyl-2-pyrrolidinone ;
(méth)acrylates d'éthers d'alcools, de préférence des (méth)acrylates d'éthers d'alcools choisis parmi le (méth)acrylate de tétrahydrofurfuryle, le (méth)acrylate de méthoxyéthoxyéthyle, le (méth)acrylate de 1-butoxypropyle, le (méth)acrylate de cyclohexyloxyéthyle, le (méth)acrylate de propoxyéthoxyéthyle, le (méth)acrylate de benzyloxyéthyle, le (méth)acrylate de furfuryle, le (méth)acrylate de 2-butoxyéthyle, le (méth)acrylate de 2-éthoxy-2-éthoxyéthyle, le (méth)acrylate de 2-méthoxy-2-éthoxypropyle, les (méth)acrylates éthoxylés, le (méth)acrylate de 1-éthoxybutyle, le (méth)acrylate de méthoxyéthyle, le (méth)acrylate de 2-éthoxy-2-éthoxy-2-éthoxyéthyle, les esters d'acide (méth)acrylique et les méthoxypolyéthylène glycols ;
(méth)acrylates d'alcools halogénés, de préférence des (méth)acrylates d'alcools halogénés choisis parmi le (méth)acrylate de 2,3-dibromopropyle, le (méth)acrylate de 4-bromophényle, le (méth)acrylate de 1,3-dichloro-2-propyle, le (méth)acrylate de 2-bromoéthyle, le (méth)acrylate de 2-iodoéthyle, le (méth)acrylate de chlorométhyle ;
(méth)acrylate d'oxiranyle, de préférence (méth)acrylate d'oxiranyle choisi parmi le (méth)acrylate de 2,3-époxybutyle, le (méth)acrylate de 3,4-époxybutyle, le (méth)acrylate de 10,11-époxyundécyle, le (méth)acrylate de 2,3-époxycyclohexyle, les (méth)acrylates d'oxiranyle tels que le (méth)acrylate de 10,11-époxyhexadécyle, le (méth)acrylate de glycidyle ;
(méth)acrylates contenant du phosphore, du bore et/ou du silicium, de préférence des (méth)acrylates contenant du phosphore, du bore et/ou du silicium choisis parmi le (méth)acrylate de 2-(diméthylphosphato)propyle, le (méth)acrylate de 2-(éthylphosphito)propyle, le (méth)acrylate de 2 diméthylphosphinométhyle, le (méth)acrylate de diméthylphosphonoéthyle, le phosphonate de diéthylméthacryloyle, le phosphate de dipropylméthacryloyle, le (méth)acrylate de 2 (dibutylphosphono)éthyle, le borate de 2,3-butylèneméthacryloyléthyle, le méthyldiéthoxyméthacryloyléthoxysiliane, le (méth)acrylate de diéthylphosphatoéthyle ;
(méth)acrylates contenant du soufre, de préférence des (méth)acrylates contenant du soufre choisis parmi le (méth)acrylate d'éthylsulfinyléthyle, le (méth)acrylate de 4-thio-cyanatobutyle, le (méth)acrylate d'éthylsulfonyléthyle, le (méth)acrylate de thiocyanatométhyle, le (méth)acrylate de méthylsulfinylméthyle, le sulfure de bis(méthacryloyloxyéthyle) ;
(méth)acrylates hétérocycliques, de préférence des (méth)acrylates hétérocycliques choisis parmi le (méth)acrylate de 2-(1-imidazolyl)éthyle, le (méth)acrylate d'oxazolidinyléthyle, la N-méthacryloylmorpholine et le (méth)acrylate de 2-(4-morpholinyl)éthyle ;
acide maléique et dérivés d'acide maléique, de préférence mono- et diesters d'acide maléique, anhydride maléique, anhydride méthylmaléique, maléinimide, méthylmaléinimide ;
acide fumarique et dérivés d'acide fumarique, de préférence mono- et diesters d'acide fumarique ;
halogénures de vinyle, de préférence des halogénures de vinyle choisis parmi le chlorure de vinyle, le fluorure de vinyle, le chlorure de vinylidène et le fluorure de vinylidène ;
esters de vinyle, de préférence acétate de vinyle ;
monomères vinyliques contenant des groupes aromatiques, de préférence des monomères vinyliques contenant des groupes aromatiques choisis parmi le styrène, les styrènes substitués par un substituant alkyle dans la chaîne latérale, tels que l'alpha-méthylstyrène et l'alpha-éthylstyrène, les styrènes substitués par un substituant alkyle sur le cycle tels que le vinyltoluène et le p-méthylstyrène, les styrènes halogénés tels que les monochlorostyrènes, les dichlorostyrènes, les tribromostyrènes et les tétrabromostyrènes ;
composés vinyliques hétérocycliques, de préférence des composés vinyliques hétérocycliques choisis parmi la 2-vinylpyridine, la 3-vinylpyridine, la 2-méthyl-5-vinylpyridine, la 3-éthyl-4-vinylpyridine, la 2,3-diméthyl-5-vinylpyridine, la vinylpyrimidine, la vinylpipéridine, le 9-vinylcarbazole, le 3-vinylcarbazole, le 4-vinylcarbazole, le 1-vinylimidazole, le 2-méthyl-1-vinylimidazole, la N-vinylpyrrolidone, la 2-vinylpyrrolidone, la N-vinylpyrrolidine, la 3-vinylpyrrolidine, le N-vinylcaprolactame, le N-vinylbutyrolactame, le vinyloxolane, le vinylfurane, le vinylthiophène, le vinylthiolane, les vinylthiazoles et les vinylthiazoles hydrogénés, les vinyloxazoles et les vinyloxazoles hydrogénés ;
éthers vinyliques et isoprényliques ;
acide méthacrylique et acide acrylique, ou un mélange de ceux-ci.

7. Composition selon l'une quelconque des revendications précédentes, dans laquelle la composition comprend de 0,001 à 1 % en poids, de préférence de 0,005 à 0,8 % en poids, plus préférablement de 0,005 à 0,5 % en poids de l'additif polymérique b), par rapport au poids total de la composition.

8. Composition selon l'une quelconque des revendications précédentes, dans laquelle le copolymère P) a un poids moléculaire moyen en poids de 8 000 à 600 000 g/mole, de préférence de 8 000 à 300 000 g/mole, encore plus préférablement de 8 000 à 100 000 g/mole et le plus préférablement de 10 000 à 50 000 g/mole, déterminé par chromatographie à perméation de gel en utilisant des étalons de poly(méthacrylate de méthyle) selon la norme DIN 55672-1.

9. Composition selon l'une quelconque des revendications précédentes, dans laquelle l'huile de pyrolyse de plastique a) est une huile de pyrolyse de plastique et/ou une huile de pyrolyse de déchets de plastique, dans laquelle la matière plastique et les déchets de plastique sont choisis parmi les polyoléfines, un poly(téréphtalate d'éthylène), un poly(chlorure de vinyle), un polystyrène ou un mélange de ceux-ci.

10. Composition selon la revendication 9, dans laquelle l'huile de pyrolyse de plastique a) comprend de 0 % à 12 % de cires n-paraffiniques en C₁₆ à C₁₉, de 0 % à 12 % de cires n-paraffiniques en C₂₀ à C₂₉, de 0 % à 12 % de cires n-paraffiniques en C₃₀ à C₃₉ et de 0 % à 12 % de cires n-paraffiniques ayant des chaînes carbonées en C₄₀ ou plus longues, la teneur totale en cire des cires n-paraffiniques ayant des chaînes carbonées en C₁₆ ou plus longues s'élevant à 12 % en poids ou moins, par rapport au poids total de l'huile de pyrolyse de plastique.

11. Composition selon l'une quelconque des revendications précédentes, dans laquelle la composition comprend en outre un additif c), dans laquelle l'additif c) est l'un quelconque du groupe comprenant les inhibiteurs d'incrustations, les inhibiteurs de corrosion, les désoxygénants, les biocides, les brise-émulsion, les agents antimousses, les agents réducteurs de traînée, les inhibiteurs d'hydrates, les dispersants paraffiniques, les agents de régulation des asphaltènes, un agent d'abaissement du point d'écoulement autre que le copolymère P), ou un mélange de ceux-ci.

12. Composition selon l'une quelconque des revendications précédentes, dans laquelle l'additif polymérique b) réduit le point d'écoulement de l'huile de pyrolyse a) d'au moins 1 °C, ou dans laquelle l'additif polymérique b) réduit la viscosité de l'huile de pyrolyse a) d'au moins 10 % à une température de - 20 °C à +80 °C, ou les deux.

13. Procédé de fabrication de la composition telle que définie dans l'une quelconque des revendications 1 à 12, comprenant les étapes de :
fourniture d'une matière première de plastique ;
pyrolyse de la matière première de plastique pour générer l'huile de pyrolyse de plastique a) ;
préparation de l'additif polymérique b) et
ajout de l'additif polymérique b) à l'huile de pyrolyse de plastique a).

14. Utilisation d'un additif polymérique b) tel que défini dans l'une quelconque des revendications 1 à 12 pour réduire le point d'écoulement d'une huile de pyrolyse de plastique a) ou pour réduire la viscosité de l'huile de pyrolyse de plastique a), ou les deux.

15. Procédé de transport ou de stockage d'une huile de pyrolyse de plastique a) comprenant l'étape d'ajout d'un additif polymérique b) à l'huile de pyrolyse de plastique a), pour former une composition telle que définie dans l'une quelconque des revendications 1 à 12.
